

# United States Patent Office.

ALFRED PARAF, OF NEW YORK, N. Y.

*Letters Patent No. 80,207, dated July 21, 1868.*

## IMPROVEMENT IN THE MANUFACTURE OF WATER-PROOF TEXTILE FABRICS.

The Schedule referred to in these Letters Patent and making part of the same.

TO ALL WHOM IT MAY CONCERN:

Be it known that I, ALFRED PARAF, now residing in the city, county, and State of New York, have invented a new and useful Article of Manufacture, which I denominate Asphalte Cloth, and that the following is a full, clear, and exact description and specification of my said invention.

My invention is based upon the discovery made by me that albumen will precipitate asphaltum or some of its component parts from its solutions, and my invention consists of the combination of a textile fabric with a coating of albuminized asphaltum, or an albuminized component of asphaltum, the said combination being a water-proof cloth applicable to a great variety of purposes in the useful arts, for which India-rubber cloths are now used.

My new combination may be produced in several ways, of which the following has been found by trial to give the best result: I use, as the basis of my new cloth, ordinary woven cotton cloth, and I treat it alternately with solutions of albumen and asphaltum, taking care to dry the fabric, by permitting it to hang in a warm room after each application of a solution. The albumen employed may be of either animal or vegetable origin, that which I prefer to use being the gluten obtained from wheat flour by the usual process of obtaining that article. In order to prepare my albuminous solution, I dissolve the gluten in dilute acetic acid, and I add a sufficient quantity of water to the solution to make it contain, when ready for use, about twenty per cent. of its weight of gluten.

In preparing the solution of asphaltum, I prefer to make use of that variety of it which is known by the name of Grahame, although others of the soluble asphaltums may be used. I dissolve one part, by weight, of Grahame in two parts, by weight, of benzole, by the aid of heat. Afterwards the solution is filtered, and from two and a half to five per cent. of its weight of the viscid solution of India rubber in benzole (commonly sold as India-rubber cement) is added to the solution, the quantity so added depending upon the suppleness which it is desired the fabric should have when finished.

The cloth is first immersed in the albuminous solution, and is then passed between squeezing-rollers to expel the surplus liquid, after which it is hung up until dry. The dry albuminized cloth is next immersed in the asphaltum-solution, or is coated with it, according to the character which the fabric is to have when finished. If it is to be coated on one side with the albuminized asphaltum, the solution of asphaltum may be applied to the albuminized cloth by means of a brush, or may be spread upon it by means of a doctor, or in the mode used in the manufacture of India-rubber cloths for spreading the solution of India rubber upon cloth. After the spreading is completed, the fabric is hung up to dry, and when dry is coated a second time (by brushing or immersion) with the albuminous solution. When this coating has become dry, the cloth is coated a second time with the solution of asphaltum, and is again dried. This duplex coating of albumen and asphaltum is generally sufficient to make the cloth impervious to water, but, if deemed expedient, the number of alternate coatings may be increased until the albuminized asphaltum has attained the desired thickness upon the face of the fabric. After the last coat of asphaltum has become dry, I subject the fabric to the action of hot calender-rolls, such as are used in print-works for calendering fabrics, and I find it expedient to heat those rolls (either by gas or by steam) to a temperature of about 200° Fahrenheit.

The above operations may be varied by applying a second thickness of albuminized cloth to the coated side of the first after the last coating of the asphaltum solution has been applied, and by subjecting the fabric to pressure before the asphaltum-solution dries, (in which case the asphalte cloth produced will have a cloth face at each side,) and by combining several thicknesses of cloth, by means of the albuminized asphaltum, heavy impervious cloth articles, such as hose for water, and machine-beltting, can be produced. Again, the character of the asphalte cloth may be varied by sifting flock, fur-clippings, or shoddy over the coated surface while the last coating of asphaltum is sticky, and by subjecting the whole to pressure between rolls, so as to compress the fibrous material into the moist asphaltum, and cause it to adhere to the fabric when it has become dry.

Although I prefer to use gluten and acetic acid for the preparation of the albuminous solution, and Gra-

hamite and benzole for the preparation of the asphaltum-solution, my invention is not restricted to these materials for the preparation of the two solutions, as the kinds of albumen and soluble asphaltum and the solvents employed may be varied as found expedient, as well as the mode in which the albuminized asphaltum is produced upon the cloth. So, also, any variety of textile fabric that is found useful may be employed as the basis of my new fabric, felted cloths being advantageous when the fabric is to be used for the manufacture of over-shoes, leggings, and many other articles of clothing.

Although I prefer to use India rubber as a constituent of the asphaltum-solution, my invention is not limited to such use, and in some cases I propose to add a small quantity of a vegetable oil, such as linseed or castor-oil, to the asphaltum-solution before applying it to the cloth.

What I claim as my invention, and desire to secure by Letters Patent, is—

The asphalte cloth hereinbefore described, consisting of the combination of a textile fabric with albuminized asphaltum, substantially as before set forth.

In testimony whereof, I have hereto set my hand, this third day of February, A. D. 1868.

ALFRED PARAF.

Witnesses:

E. S. RENWICK,  
J. RATHBONE, Jr.